

## 1

3,689,272

PHOTOGRAPHIC COLOR PROCESSES WHICH  
YIELD EITHER POSITIVE OR NEGATIVE  
SILVER-TRANSFER IMAGES

Judith A. Schwan and Edward A. Smith, Rochester, N.Y.,  
assignors to Eastman Kodak Company, Rochester, N.Y.  
No Drawing. Filed Jan. 25, 1971, Ser. No. 109,719  
Int. Cl. G03c 5/54, 7/02, 5/44

U.S. Cl. 96—3

19 Claims

## ABSTRACT OF THE DISCLOSURE

Photographic color elements having a support coated on one side with at least one light-sensitive hydrophilic colloid layer containing imagewise-exposed silver halide grains and a nondiffusible coupler that reacts with oxidized aromatic primary amine color developing agent to form a nondiffusible dye, are advantageously processed by (1) contacting with a hydrophilic colloid processing web containing silver precipitating nuclei, an aromatic primary amine color developing agent, an organic amine-SO<sub>2</sub> addition product and, alternatively, an additional silver halide solvent until a dye image and silver image are formed in the element and a silver image is formed in the processing web, (2) separating the processing web from the element and, if desired, subsequently treating the element to remove silver and residual silver halide, provided that the hydrophilic colloid in the element and the hydrophilic colloid in the processing web are either hardened during manufacture or during step (1) by a hardener imbibed in the processing web just prior to step (1) to have a reticulation temperature greater than 65° C. and a melting point greater than 85° C.

This invention is related to photography and more particularly to color photographic processing.

In the well-known silver halide diffusion transfer process of photography, an exposed emulsion layer is developed in the presence of a silver halide solvent, the emulsion layer being for at least a portion, or for the whole of the development period, in effective contact with a receiving sheet, the surface of which generally carries a quantity of a silver precipitant which comprises either physical development nuclei such as colloidal silver or silver sulfide or a chemical precipitant for silver ions, such as zinc sulfide. Development of the emulsion layer proceeds accompanied by complexing of the residual unexposed and undeveloped silver halide with a silver halide solvent also present in the developer composition, and imagewise diffusion of the resulting silver complex to the receiving sheet where the silver precipitant causes the formation of an argental image.

This process has been applied successfully to a large variety of black-and-white films of all types, ranging from low speed recording and printing films to the highest speed negative films. However, no successful application of diffusion transfer processing to conventional color films has been achieved. There exists a need of a process for a color film that will produce a quick access black-and-white transfer image in a processing web, and at the same time allow the production of a color dye image in the color film.

It is an object of this invention to provide a novel, simplified process for obtaining a black-and-white image from a color film, while simultaneously developing a dye image in the color film.

Another object of this invention is the provision of a novel process for a color film that is essentially free of excess liquid in the color development step.

These and still other objects are accomplished by use of the color process of our invention. Our color process

## 2

is advantageously used for an imagewise-exposed photographic element for producing a silver image and a nondiffusible color (i.e., dye) image in the element and simultaneously producing a corresponding transfer silver image in a hydrophilic colloid processing web coated on a separate support. The photographic element comprises a support coated with at least one hydrophilic colloid layer containing dispersed silver halide grains [preferably camera speed (e.g., ASA speed of from 5 to 5000) silver bromoiodide grains] and a nondiffusible dye-forming coupler that reacts with an oxidized aromatic primary amine color developing agent to produce a nondiffusible dye. The hydrophilic colloid processing web and hydrophilic colloid emulsion layers are either hardened during manufacture or during the web processing step by a hardening agent imbibed in the processing web so they each have a reticulation temperature greater than 65° C. and a melting point greater than 85° C., determined by observing the hydrophilic colloid layer on a sample strip immersed in a mechanically stirred distilled water bath at 23° C. as it is heated to give a 3.3° C. temperature rise per minute up to 100° C. (maintained for 2 minutes), the reticulation temperature being the bath temperature at which the layer shows the first sign of reticulation and the melting point being the bath temperature at which the layer shows the first evidence of stripping, sloughing off or frilling (in areas >1.5 mm. from the edge of sample). Our process comprises the steps:

- (1) contacting the hydrophilic colloid layer of the photographic element with the hydrophilic colloid processing web which contains silver precipitating agent, an alkali, an aromatic primary amine color developing agent and a silver halide solvent until substantially all of the developable silver halide grains (i.e., exposed grains in color negative emulsions or unexposed grains in color direct-positive emulsions) in the photographic element are developed to a silver and a nondiffusible dye image, and at least a part of the residual undeveloped silver halide grains in areas not color developed in the photographic element are dissolved by the silver halide solvent and transferred imagewise to the hydrophilic colloid processing web where a silver image is formed on the silver precipitating agent, the processing web containing a sufficient amount of a hardening agent to harden both web and hydrophilic colloid layers of the element when these layers are not hardened during manufacture; and
- (2) separating the processing web containing the silver image from the photographic element containing the silver and dye image and any residual undeveloped silver halide.

Usually, the process is continued to remove the silver image and any residual silver halide so that the dye image is unobstructed and made permanent by following step (2) with steps (3) and (4) or alternatively step (5) is used in place of steps (3) and (4).

- (3) contacting the silver image and any residual silver halide in the photographic element with a silver bleach bath comprising a photographic silver oxidizing agent (e.g., an alkali metal ferricyanide, an alkali metal dichromate, quinone, etc.) until the silver is converted to a silver salt; and
- (4) contacting the silver salt(s) with a photographic fixing bath comprising a silver salt solvent (e.g., an alkali metal or ammonium thiosulfate, an alkali metal or ammonium thiocyanate, thiourea, etc.) until the silver salt(s) is dissolved and diffuses from the photographic element;
- (5) contacting the silver image and any residual silver halide in the photographic element from step (2) with a combined bleach-and-fix solution comprising a silver oxidizing agent [e.g., an alkali metal ferricyanide, a

salt with an unchelated cation (e.g., alkali metal or ammonium) and an anion that is  $\text{Fe}^{+++}$ ,  $\text{Co}^{+++}$  or  $\text{Cu}^{++}$  chelated with a polyfunctional ligand (e.g., a polycarboxylic or polyphosphoric acid chelating agent), such as, sodium or ammonium ethylenedinitrilotetraacetato ferrate (III), sodium ethylenedinitrilotetraacetato cobaltate (III), ammonium ethylenedinitrilotetraacetato cuprate (II), etc.] and a silver salt solvent, e.g., an alkali metal or ammonium thiosulfate, an alkali metal or ammonium thiocyanate, etc. until the silver and silver salt(s) is dissolved and diffuses from the photographic element.

The hydrophilic colloid processing web used in step (1) contains dispersed silver precipitating agent, and at the time of contact with the image-exposed photographic element, sufficient processing solution to develop substantially all the developable silver halide, and to simultaneously form a color dye image in emulsion layer(s) of the photographic element. The processing solution contains an aromatic primary amine color developing agent, an organic amine  $-\text{SO}_2$  addition product and, optionally, additional silver halide solvent and where necessary a hardening agent. The processing solution also advantageously contains a suitable toning agent or combination of toning agents. The processing web is maintained in intimate contact with the outermost hydrophilic colloid layer of the photographic element until development of developable silver halide is substantially complete, a dye image is formed in each of the exposed layers of the color photographic element, and at least a portion of the undeveloped silver halide has been dissolved from the emulsion layers and deposited in the processing web to form a black-and-white image. Precipitating agents for the purpose of this invention are either nuclei or development centers on which silver from a suitable silver halide complex is precipitated as metallic silver by physical development, or compounds which react with silver of the soluble silver halide complex to form an insoluble silver compound. The processing element is then separated from the substantially completely developed emulsion, which requires only a bleaching and fixing operation, or combined bleaching and fixing, followed by water washing, to render the color dye image permanent.

The color photographic element comprises a support having at least one hydrophilic colloid silver halide emulsion layer containing a nondiffusible dye-forming coupler that reacts with oxidized aromatic primary amine color developing agent to form a nondiffusible dye image. Usually, the elements are multilayer, multicolor and contain a first hydrophilic colloid silver halide emulsion layer sensitive to light from a first region of the visible spectrum and a coupler that reacts with oxidized aromatic primary amine color developing agent to form a nondiffusible dye image of a first color, a second hydrophilic colloid silver halide emulsion layer sensitive to a second region of the visible spectrum that is different from the first region and a second coupler that reacts with oxidized aromatic primary amine color developing agent to form a nondiffusible dye image of a second color that is different from the first color dye, and a third hydrophilic colloid silver halide emulsion layer sensitive to a third region of the visible spectrum that is different from the first and second regions and a third coupler that reacts with oxidized aromatic primary amine color developing agent to form a nondiffusible dye image of a third color that is different from the first color and the second color. Preferably the hydrophilic colloid layers are hardened during manufacture. Usually, the dye-forming coupler is selected for a given silver halide emulsion so that it forms, upon reaction with oxidized color developing agent, a dye having a color that is complementary to the color of the light to which the silver halide emulsion is sensitive. Thus, a phenol or a naphthol cyan-dye-forming coupler is usually incorporated in a red-sensitive silver halide emulsion layer; a 5-pyrazolone or a 1H-pyrazolo-

[3,2-c]-s-triazole magenta-dye-forming coupler is usually incorporated in a green-sensitive silver halide emulsion layer; and an open-chain yellow-dye-forming coupler is incorporated in a blue-sensitive silver halide emulsion layer. These differently sensitive silver halide emulsion layers are advantageously arranged on one side of a support in any order desired. Particularly advantageously orders are with the support coated in succession with a red-sensitive layer, a green-sensitive layer and a blue-sensitive layer, and with the support coated in succession with a blue-sensitive layer, a green-sensitive layer and a red-sensitive layer. The photographic elements advantageously contain additional layers, for example, a second red-sensitive layer contiguous to the first red-sensitive layer, a second green-sensitive layer contiguous to the first green-sensitive layer, a second blue-sensitive layer contiguous to the first blue-sensitive layer, non-sensitive, hydrophilic colloid light-filtering interlayers, etc. In photographic elements having the blue-sensitive layer farthest from the support, it is advantageous to have a layer with a bleachable yellow-colored blue-light-absorbing material between the blue-sensitive layer and the light-sensitive layer under it. Photographic elements used to advantage in our process include those described by Froehlich et al., U.S. Pat. 2,376,679; Vittum et al., U.S. Pat. 2,322,027; Fierke et al., U.S. Pat. 2,801,171; Godowsky, U.S. Pat. 2,698,794; Barr et al., U.S. Pat. 3,227,554; Graham, U.S. Pat. 3,046,129 and Wolf et al., U.S. Pat. 3,516,831. Other photographic elements used to advantage in the process of our invention have the differently sensitive silver halide grains coated in a single hydrophilic colloid layer so that, for example, this layer contains a dispersion of minute particles containing red-sensitive silver halide grains and cyan-dye-forming coupler, a dispersion of minute particles containing green-sensitive silver halide grains and magenta-dye-forming coupler and a dispersion of minute particles containing blue-sensitive silver halide grains and yellow-dye-forming coupler as has been described by references such as Martinez, U.S. Pat. 2,284,877.

In one embodiment, our process is used to produce in a color negative element and a web, a color negative and a silver positive, respectively, and in another embodiment our process is used to produce in a direct color reversal element and a web, a color positive and a silver negative, respectively.

Any of the photographic silver halide emulsions, e.g., silver bromide, silver bromoiodide, silver chloride, silver chlorobromide, silver bromochloroiodide, etc., used in photography are used to advantage in the color elements used in our process including negative and direct-positive emulsions. The direct-positive emulsions advantageously comprise reduction and gold-fogged, cubic-shaped, silver halide grains having a uniform diameter frequency distribution with an average grain size in the range of from about 0.01 to about 2 microns, comprising at least about 50 mole percent bromide and preferably silver bromoiodide emulsions containing less than 10 mole percent iodide, as described in columns 2 through 8 in Illingsworth, U.S. Pat. 3,501,305, issued Mar. 17, 1970.

The emulsions used in the photographic elements are advantageously chemically sensitized by any of the accepted procedures. The emulsions can be digested with naturally active gelatin, or sulfur compounds can be added, such as those described in Sheppard, U.S. Pat. 1,574,944, issued Mar. 2, 1926; Sheppard et al., U.S. Pat., 1,623,499, issued Apr. 5, 1927; and Sheppard et al., U.S. Pat. 2,410,689, issued Nov. 5, 1946.

The emulsions can also be treated with salts of the noble metals, such as ruthenium, rhodium, palladium, iridium and platinum, as described in Smith et al., U.S. Pat. 2,448,060, issued Aug. 31, 1948 and as described in Trivelli et al., U.S. Pats. 2,566,245 and 2,566,263, both issued Aug. 28, 1951.

The emulsions are advantageously spectrally sensitized with cyanine and merocyanine dyes, such as those de-

scribed in Brooker, U.S. Pats. 1,846,301 and 1,846,302, both issued Feb. 23, 1932; and 1,942,854, issued Jan. 9, 1934; White, U.S. Pat. 1,990,507, issued Feb. 12, 1935; Brooker and White, U.S. Pats. 2,112,140, issued Mar. 22, 1938; 2,165,338, issued July 11, 1939; 2,493,747, issued Jan. 10, 1950; and 2,739,964, issued Mar. 27, 1956; Brooker et al., U.S. Pat. 2,493,748, issued Jan. 10, 1950; Sprague, U.S. Pats. 2,503,776, issued Apr. 11, 1950 and 2,519,001, issued Aug. 15, 1950; Heseltine et al., U.S. Pat. 2,666,761, issued Jan. 19, 1954; Heseltine, U.S. Pat. 2,734,900, issued Feb. 14, 1956; Van Lare, U.S. Pat. 2,739,149, issued Mar. 20, 1956; and Kodak Limited, British 450,958, accepted July 15, 1936.

The emulsions advantageously contain speed-increasing compounds of the quaternary ammonium type of Carroll, U.S. Pat. 2,271,623, issued Feb. 3, 1942; Carroll et al., U.S. Pat. 2,288,226, issued June 30, 1942; and Carroll et al., U.S. Pat. 2,334,864, issued Nov. 23, 1943; and the polyethylene glycol type of Carroll et al., U.S. Pat. 2,708,162, issued May 10, 1955.

The emulsions are advantageously chemically sensitized with gold salts as described in Waller et al., U.S. Pat. 2,399,083, issued Apr. 23, 1946, or stabilized with gold salts as described in Damschroder, U.S. Pat. 2,597,856, issued May 27, 1952; and Yutzy et al., U.S. Pat. 2,597,915, issued May 27, 1942. Suitable compounds are potassium chloroaurite, potassium aurithiocyanate, potassium chloroaurate, auric trichloride and 2-aurosulfobenzothiazole methochloride.

Hydrophilic colloids used to advantage include gelatin, colloidal albumin, a cellulose derivative, or a synthetic resin, for instance, a polyvinyl compound. Some colloids which are advantageously used are polyvinyl alcohol or a hydrolyzed polyvinyl acetate as described in Lowe, U.S. Pat. 2,286,215, issued June 16, 1942; a far hydrolyzed cellulose ester, such as cellulose acetate hydrolyzed to an acetyl content of 19-26% as described in Lowe et al., U.S. Pat. 2,327,808, issued Aug. 24, 1943; a water-soluble ethanolamine cellulose acetate as described by Yutzy, U.S. 2,322,085, issued June 15, 1943; a polyacrylamide having a combined acrylamide content of 30-60% and a specific viscosity of 0.25-1.5 or an imidized polyacrylamide of like acrylamide content and viscosity as described in Lowe et al., U.S. Pat. 2,541,474, issued Feb. 13, 1951; zein as described in Lowe, U.S. Pat. 2,563,791, issued Aug. 7, 1951, a vinyl alcohol polymer containing urethane carboxylic acid groups of the type described in Unruh et al., U.S. Pat. 2,768,154, issued Oct. 23, 1956, or containing cyano-acetyl groups, such as the vinyl alcohol-vinyl cyano-acetate copolymer as described in Unruh et al., U.S. Pat. 2,808,331, issued Oct. 1, 1957; or a polymeric material which results from polymerizing a protein or a saturated acylated protein with a monomer having a vinyl group as described in Illingsworth et al., U.S. Pat. 2,852,382, issued Sept. 16, 1958.

The hydrophilic colloids described above are used in various layers of the photographic elements. The hydrophilic colloid layers are hardened either during manufacture or during the web processing step sufficiently so that their reticulation temperature and melting points, as defined herein previously, are higher than 65° C. and higher than 85° C., respectively, with hardening agents, such as aziridine hardeners, oxazolium hardeners, vinyl sulfone hardeners, mucochloric acid, aldehyde hardeners, e.g., glutaraldehyde, glutaraldehyde bisulfite, succinaldehyde, formaldehyde, epoxy ether hardeners, e.g., bis (2,3-epoxypropoxyethyl)ether, etc. The aziridine hardeners used to advantage include 1,3-bis(1-aziridinylsulfonyl)-propane, 1-(1-aziridinyl carbonyl)-3-(1-aziridinylsulfonyl)-benzene and others described in Burness, U.S. Pat. 2,964,404, issued Dec. 13, 1960; N,N-trimethylene-bis(1-aziridine-carboxamide), N,N'-octamethylene-bis(1-aziridine-carboxamide), toluene-2,4-bis(1-aziridine-carboxamide), N,N-tetramethylene bis(1-aziridine-carboxamide) and others described in Allen and Webster,

U.S. Pat. 2,950,197, issued Aug. 23, 1960; and the aziridinyl azine hardener compounds prepared by reacting cyanine chloride with ethylene imine as described by Yudelson, U.S. Pat. 3,017,280, issued Jan. 16, 1962. The oxazolium hardeners used to advantage include 2,5-dimethylisoxazolium perchlorate, 2-ethyl-5-phenylisoxazolium-3'-sulfonate and others described in Van Campen and Graham, U.S. Pat. 3,316,095, issued Apr. 25, 1967, 2-methylisoxazolium-p-toluenesulfonate, 3-(2-isoxazolium)propanesulfonate, 2,5-dimethylisoxazolium-p-toluenesulfonate, 2-methyl-5-phenylisoxazolium perchlorate, 4-(3-hydroxypropyl)-2-methylisoxazolium-p-toluenesulfonate, 5-isopropyl-2-methylisoxazolium perchlorate, 2,4-dimethylisoxazolium-p-toluenesulfonate, 3-[2-(5-methylisoxazolium)]propanesulfonate described by Burness and Wilson, U.S. Pat. 3,321,313, issued May 23, 1967. The vinylsulfones used to advantage as hardeners for hydrophilic colloids in our photographic elements include hardening compounds having two vinylsulfonylalkyl groups linked to a single linking heteroatom (e.g., nitrogen atom, or oxygen atom) or radical, including hardeners such as, bis(4-vinylsulfonylbutyl)ether, bis(2-vinylsulfonylethyl)ether, bis(vinylsulfonylmethyl)ether, N,N-bis(2-vinylsulfonylethyl)-N-propylamine, N,N-bis(2-vinylsulfonylethyl)-N-ethyl-N-propylammonium tetrafluoroborate, and bis(1-vinylsulfonylethyl)ether, etc., and other compounds of the formula:



in which  $m_2$  is an integer of from 1 to 4,  $Z^{00}$  is a heteroatom (e.g., nitrogen or oxygen) and  $R^6$  is hydrogen, or lower alkyl groups (e.g., methyl, ethyl, isopropyl, etc., which can in turn be further substituted), and hardening compounds having two or more vinylsulfonylalkyl groups (i.e., lower alkyl from 1 to 4 carbon atoms) attached to a plurality of tertiary or quaternary atoms and/or a plurality of ether oxygen atoms including typical compounds, such as:

- (1) N,N-bis(2-vinylsulfonylethyl)piperazine
- (2) N,N-bis(2-vinylsulfonylethyl)piperazine-bis(metho-perchlorate)
- (3) N,N'-bis(2-vinylsulfonylethyl)-N,N'-dimethyl-2-betene-1,4-diamine bis(metho-p-toluenesulfonate) and the corresponding bis(methofluoroborate)
- (4) N,N'-bis(2-vinylsulfonylethyl)-N,N'-dimethyl-ethylene bis(metho-p-toluenesulfonate)
- (5) 1,2-bis(vinylsulfonylmethoxy)ethane
- (6) 1,4-bis(2-vinylsulfonylethoxy)butane
- (7) bis[2-(2-vinylsulfonylethoxy)ethyl]sulfone
- (8) N,N'-bis[2-(2-vinylsulfonylethoxy)ethyl]urea
- (9) 1,14-bis(vinylsulfonylethoxy)-3,6,9,12-tetraoxatetradecane

as are described in Belgian Pat. 686,440, granted Nov. 14, 1966 and Belgian Pat. 723,806, granted Jan. 15, 1969.

The light-sensitive layers of the photographic elements are advantageously coated on a wide variety of photographic emulsion supports. Typical supports used to advantage include cellulose nitrate film, cellulose acetate film, polyacetal film, polystyrene film, poly(ethylene-terephthalate) film, polyethylene film and related films of resinous materials as well as paper, glass and others.

Any of the non-diffusible color-forming couplers used in photographic elements are used to advantage in the photographic elements for our process. Included among the phenol and naphthol cyan-dye-forming couplers used to advantage are those described by the following U.S. patents: 2,423,730, 2,474,293, 2,521,908, 2,725,291, 2,801,171, 3,253,294, etc. Included among the keto-methylene yellow-dye-forming couplers used to advantage are those described in U.S. Pats. 2,298,443, 2,778,658, 2,801,171, 2,875,057, 3,253,924, 3,277,155, etc. Included 75 among the 5-pyrazolone magenta-dye-forming couplers

used to advantage are those described in U.S. Pats. 2,600,788, 2,801,171, 3,252,924, etc.

Dispersing agents for color-forming couplers and the dispersing techniques used to advantage include those set forth in Jelley et al., U.S. Pat. 2,322,027; Mannes et al., U.S. Pat. 2,304,940; Fierke et al., U.S. Pat. 2,801,171, etc.

The processing elements or processing webs of the present invention comprise a hydrophilic organic colloid layer containing dispersed silver precipitating agent. The hydrophilic layers are employed alone if they have sufficient strength to be self-supporting, or if desired, they are coated on suitable supports. The supports and any subbing layers are preferably inert to the chemicals in the processing solution, and it is desirable in some cases that such supports be hydrophobic in nature as well. Suitable hydrophilic organic colloids include gelatin, cellophane, poly(vinyl alcohol), sulfonated poly(vinyl alcohol) derivatives [e.g., copolymers prepared from poly(vinyl alcohol) and sodium 2-sulfobenzaldehyde, copolymers prepared from poly(vinyl alcohol) and sodium 2-sulfobenzaldehyde and cyanoacetamidoacetaldehyde diethyl acetal, copolymers prepared from poly(vinyl alcohol) and sodium 4-methoxy-3-sulfobenzaldehyde, copolymers prepared from poly(vinyl alcohol) and 2,4-disulfobenzaldehyde, etc.], hydrolyzed cellulose acetate, cellulose ether phthalate, carboxylated rubber and similar materials. Particularly useful hydrophilic materials are gelatin and a copolymer made up of 80 percent acrylic acid and 20 percent ethyl acrylate. The hydrophilic colloid layer of the processing web is hardened so that its reticulation temperature and its melting point are higher than 65° C. and higher than 85° C., respectively (when measured as described herein previously) with any of the hardening agents described herein previously for hardening the hydrophilic colloid layers of the photographic element. For best results in operating our process, it is advantageous to select hydrophilic colloids for the processing web that will adhere well to the hydrophilic colloid in the emulsion layers of the photographic element during the first step of our process, but which separate readily from the processed film in Step 2.

The silver precipitating agents incorporated in the hydrophilic colloid layer of the processing webs are physical development nuclei or chemical precipitants including (a) heavy metals, especially in colloidal form, and the salts of these metals; (b) salts, the anions of which form a silver salt less soluble than the silver halide of the photographic emulsion to be processed; or (c) non-diffusing polymeric materials with functional groups capable of combining with and insolubilizing silver ion. Suitable silver precipitating agents for use in the invention are disclosed in Rott, U.S. Pat. 2,352,014, Yutzy and Yackel, U.S. Pat. 2,740,717 and in Yackel et al., U.S. Pat. 3,020,155. More specifically, useful silver precipitating agents include sulfides, selenides, polysulfides, polyselenides, thiourea and its derivatives, mercaptans, stannous halides, silver, gold, platinum, palladium, and mercury, colloidal sulfur, aminoguanidine sulfate, aminoguanidine carbonate, arsenous oxide, sodium stannite substituted hydrazines, xanthates, and the like. Polyvinyl mercaptoacetate is an example of a non-diffusing polymeric silver precipitant. Heavy metal sulfides such as lead, silver, zinc, nickel, antimony, cadmium and bismuth sulfides are useful, particularly the sulfides of lead and zinc alone or in admixture, or complex salts of these with thioacetamide, dithioxamide, or dithio-biuret. The heavy metals and the noble metals particularly in colloidal form are especially effective. Other silver precipitating agents will occur to those skilled in the art. The average particle size of these silver precipitating agents is advantageously in the range of from 7 to 2500 angstrom units. The processing web advantageously has in the range of from about 3 mg./m.<sup>2</sup> to about 1290 mg./m.<sup>2</sup> of silver precipitating agent coated in it.

The processing elements or webs of the invention take any suitable form or shape. For example, they consist of

pads, sheets, strips or webs of hydrophilic material either unsupported or coated on suitable supports such as glass, metal, paper, polyethylene, polypropylene, polystyrene, polyethylene terephthalate, cellulose esters, or the like. An especially useful web for producing reflection transfer images is that disclosed in U.S. Pat. 3,415,647.

Preferred processing solution imbibants comprise one or more aromatic primary amine color developing agents, an amine sulfur dioxide addition product, and optionally, an additional silver halide solvent, water and, when necessary, a hardening agent.

Aromatic primary amine color developing agents useful in the practice of our invention are p-phenylenediamine derivatives, such as, those given in Bent et al., J. Am. Chem. Soc., 73, 3100 (1951). Especially preferred agents are:

4-amino-3-methyl-N-ethyl-N-β-hydroxyethylaniline sulfate,  
4-amino-3-methoxy-N-β-hydroxyethylaniline hydrochloride  
4-amino-N-ethyl-N-β-hydroxyethylaniline hydrochloride,  
4-amino-3-methyl-N-ethyl-N-β-sulfoethylaniline,  
4-amino-N-ethyl-N-β-γ-dihydroxypropylaniline and  
4-amino-N-ethyl-N-(2-methoxyethyl)-m-toluidine dihydrochloride.

An operable range of developing agent concentration is from about 2 g. to about 100 g./l. and a preferred range is from about 10 g. to about 50 g./l.

Organic amine —SO<sub>2</sub> addition products used to advantage to provide alkali and silver halide solvent are prepared by reacting sulfur dioxide and an amine of the formula:



wherein R and R<sub>1</sub> each represent a member independently selected, such as hydrogen, methyl, ethyl, aminoethyl, hydroxyethyl and together they represent the nonmetallic atoms required to complete a morpholino group or a piperidino group and R<sub>2</sub> represents a member such as hydrogen, 2-hydroxyethyl, 1-methyl-2-hydroxyethyl, 1,1-dimethyl-2-hydroxyethyl and 5-hydroxypentyl such that no more than two of R, R<sub>1</sub> and R<sub>2</sub> represent hydrogen. Typical amines used in the addition products include 2-aminoethanol, 2-methylaminoethanol, 2-dimethylaminoethanol, 2-ethylaminoethanol, 2-diethylaminoethanol, 2,2'-2"-nitri-  
lotriethanol, 2-(2-aminoethylamino)ethanol, 2,2'-iminodiethanol, 5-diethylamino-2-pentanol, 2-amino-2-methyl-1-propanol, morpholine and piperidine, among others.

A preferred amine-sulfur dioxide addition product is prepared in the following manner. Sulfur dioxide gas is slowly bubbled through one mole of the preferred amine, 2-methylaminoethanol, with adequate stirring until it absorbs the equivalent of 0.5 mole of sulfur dioxide. The resulting 2-methylamino-ethanol-sulfur dioxide addition product contains the equivalent of 30 percent sulfur dioxide, by weight, or 33 mole percent. It will be understood that the ratio of SO<sub>2</sub> to amine can be increased or decreased from that just given as required to bring the pH of the processing solution to the desired level. An operable amine—SO<sub>2</sub> concentration range is from about 5 ml. to about 300 ml./l. with from about 2.5% to 35% by weight SO<sub>2</sub> and a preferred range is from about 10 ml. to about 200 ml./l. with from about 5% to about 33% by weight SO<sub>2</sub>. These compounds usually supply the alkali needed as well as supply at least a part of the silver halide solvent.

The processing solution preferably has a relatively low salt content so that it is readily absorbed by the hydrophilic colloid layers for processing. The developing capability of the processing solution is preferably relatively high in capacity and rate so development is essentially completed

before any appreciable transfer of complexed silver to the processing web occurs.

While one can incorporate a silver halide solvent, such as, up to about 50 g./l. of an alkali metal thiosulfate (e.g., sodium thiosulfate, potassium thiosulfate, etc.), an alkali metal thiocyanate (e.g., sodium thiocyanate, potassium thiocyanate, etc.), an alkali metal selenocyanate, thioglycerol, aminoethanethiols, p,p'-dithiasuberic acid, etc. in the processing solution to assist in the transfer of the complexed silver to the processing web, it is advantageous to produce the transfer silver image in the web by the use of the solvent action of the amine-sulfur dioxide addition product, and the solvent action of the p-phenylenediamine-type developing agent included. Alkali metal hydroxides, carbonates or borates are sometimes used as the alkali.

The pH of the developer solution is advantageously in the range of from about 8.5 to about 11.5 and preferably in the range of from about 9 to 11.

Toning agents suitable for incorporation in the processing solution to increase the neutrality of image tone of the image transferred to the processing web, either alone or in combination with certain onium compounds, include those described in U.S. Pats. 3,017,270 and 3,314,789. When toning agents are desired it is advantageous to use them in the concentration range of from about .002 to about 1.0 g./l. and preferably in the range of from about .01 to .25 g./l., and when onium compounds are desired, they are used in the concentration range of from about .05 to about 2.0 g./l. and preferably in the range of from about .1 to about 1.0 g./l.

The processing solution containing the aromatic primary amine color developing agent, the alkali, and silver halide solvent is imbibed into the hydrophilic colloid layer containing the silver precipitating nuclei prior to contacting the web and the light-exposed color negative element. It is advantageous to imbibe in the range of from about 48 g. to about 215 g. of the processing solution per m.<sup>2</sup> of the processing web, and preferably in the range of from about 65 g. to about 100 g. of solution per m.<sup>2</sup> of the web. Imbibition usually takes in the range of from 1 minute to 30 minutes in the range of temperature from about 20° C. to about 50° C. A minimum amount of water or moisture is utilized in the imbibed processing solution to facilitate the physical handling of the web, but sufficient in amount to effect the photographic processing reactions.

An operable web processing time is in the range of from about 3 to 60 minutes with a preferred range of from about 5 to about 20 minutes.

The process is carried out at temperatures in the range of from about 20 C. up to about 38° C., the temperature not being particularly critical. It is found, however, that even at ambient temperature (20° C.), conventional color films exhibit physical damage under the processing conditions involved in web processing and cannot be used unless a sufficient amount of a hardening agent is imbibed in the processing web to harden the hydrophilic colloid layers of element and web while they are laminated so that their reticulation temperature is greater than 65° C. and their melting point is greater than 85° C. by the time the element and web are to be separated from each other. The preferred color elements used for our process have hydrophilic colloid layers hardened sufficiently during manufacture to have reticulation temperatures above 65° C. and melting points above 85° C. (when measured in distilled water as defined herein previously), and do not exhibit any physical damage from our web process.

In processing multilayer color negative films by the process of our invention, it is found desirable for obtaining optimum transfer of complexed silver to the nuclei-containing processing web to use negative films that do not contain layers bearing particulate silver. Such silver layers are commonly used as filter layers and as antihalation layers in multilayer color films. The particulate silver in such layers tends to act as precipitating centers for the silver in the silver complexes formed by reaction of the processing solutions described herein with unexposed silver.

halide, thus preventing a portion of the complexed silver from diffusing to the processing web to form the desired argental image in the web. It will be understood, however, that the use of multilayer color films containing layers bearing particulate silver is not excluded in the present invention.

The following examples are included for a further understanding of our invention:

#### EXAMPLE 1

A multilayer color negative film hardened with bis[2-(2-vinylsulfonylethoxy)ethyl]sulfone is prepared as follows: On a cellulose acetate photographic film support, the following layers are coated, beginning at the support:

- 10 (1) A gray-colored gelatin antihalation layer containing bleachable dye.
- 20 (2) A gelatin layer.
- 25 (3) A red-sensitive silver bromoiodide gelatin photographic emulsion containing a nondiffusible cyan-dye-forming coupler that reacts with oxidized color developing agent to produce a nondiffusible cyan dye.
- 30 (4) A gelatin interlayer.
- 35 (5) A green-sensitive silver bromoiodide gelatin photographic emulsion containing a nondiffusible magenta-dye-forming coupler that reacts with oxidized color developing agent to produce a nondiffusible magenta dye.
- (6) A gelatin layer containing a yellow-colored filter dye.
- (7) A blue-sensitive silver bromoiodide gelatin photographic emulsion containing a nondiffusible yellow-dye-forming coupler that reacts with oxidized color developing agent to produce a nondiffusible yellow dye.
- 35 (8) A gelatin overcoat.

The gelatin layers are hardened so that the reticulation temperature and the melting point measured as defined herein previously are 83° C. and greater than two minutes at 100° C., respectively. The film just described is exposed to an original light image and developed in contact with a web of the following composition: A polyethylene terephthalate support is coated with gelatin at 20.4 g./m.<sup>2</sup> containing as silver precipitating nuclei 9.7 mg./m.<sup>2</sup> of nickel sulfide and 9.7 mg./m.<sup>2</sup> of silver iodide prepared as described in Example 1 of British Pat. 1,080,781. A spreading agent and hardener bis[2-(2-vinylsulfonylethoxy)ethyl]sulfone are included in the coating so that it has a reticulation temperature and a melting point measured as described previously of greater than 65° C. and greater than 85° C., respectively. The web is soaked in the following imbibant solution for ten minutes at 38° C. to imbibe about 86 g. of the solution per m.<sup>2</sup>.

55 2-methylaminoethanol-SO<sub>2</sub> addition product --ml-- 100  
4 - amino-3-methyl-N-ethyl-N-β-hydroxyethylaniline sulfate ----- g-- 40  
Sodium thiosulfate ----- g-- 10  
Water to make 1 liter.

60 pH=about 10.

After a processing period of fifteen minutes at about 20° C., the films are separated and treated as follows: The web is washed and dried, producing a good quality, positive argental transfer image reproduction of the original image. The negative color film is treated in acetic acid stop bath for thirty seconds, bleached for five minutes in a bleach having the composition:

|                                  | G.    |
|----------------------------------|-------|
| Sodium bromide -----             | 34.0  |
| Sodium sulfate (anhydrous) ----- | 120.0 |
| Potassium ferricyanide -----     | 144.0 |
| Sodium hydroxide -----           | 0.05  |
| Water to make 1 liter.           |       |

## 11

fixed for five minutes in an acid hardening fixer having the composition:

|                            |     |       |
|----------------------------|-----|-------|
| Sodium thiosulfate         | g.  | 240.0 |
| Sodium sulfite, desiccated | g.  | 15.0  |
| Acetic acid, 28%           | ml. | 48.0  |
| Boric acid, crystals       | g.  | 7.5   |
| Potassium alum             | g.  | 15.0  |
| Water to make 1 liter.     |     |       |

washed and dried to yield a three-color dye image. The processed negative color film is printed onto a reflection color print material using conventional techniques to produce upon conventional color processing a print of excellent color fidelity and definition.

## EXAMPLE 2

Example 1 is repeated, except that a water wash is used in place of the acetic acid short-stop to treat the color negative film just prior to the bleaching step. An excellent color negative is produced that is used to produce an excellent color print.

## EXAMPLE 3

An imagewise exposed sample of the color negative film described in Example 1 is developed in contact with a web of the same composition as described in Example 1 which is soaked in the followed imbibant solution for one minute at 38° C.:

|                                                                                 |     |    |
|---------------------------------------------------------------------------------|-----|----|
| 2 - methylaminoethanol - SO <sub>2</sub> addition product (7% SO <sub>2</sub> ) | ml. | 90 |
| 4-amino - 3 - methoxy-N-β-hydroxyethylaniline hydrochloride                     | g.  | 15 |
| Water to make 1 liter.                                                          |     |    |

pH=about 10.1.

The web is found to contain about 80 g. of the imbibant per m.<sup>2</sup> following the 1-minute soak. After a processing period of ten minutes at about 20° C., the films are separated as in Example 1 to give in the web a good positive black-and-white image reproduction and in the photographic element an excellent color negative and silver negative image reproduction. The photographic element is water washed, then bleached and fixed as described in Example 1 to remove the silver image and residual silver halide and leave a permanent three-color negative image reproduction of the original. This color negative is then printed onto a reflection print element as described in Example 1 to give upon conventional color processing an excellent color print reproduction of the original light image.

## EXAMPLE 4

Examples 1, 2 and 3 are repeated, but using a processing web as described in Example 1 of U.S. Pat. 3,415,647 is used in place of the film support used in immediate Examples 1, 2 and 3. Good reflection positive black-and-white reproductions are obtained in the processing web and excellent color negatives in the processed photographic element that are used to produce high quality color prints.

## EXAMPLE 5

Example 1 is repeated, but imbibing in the processing web a processing solution from which the sodium thiosulfate is omitted. An excellent black-and-white positive is obtained in the processing web and an excellent color negative is obtained in the color negative element. Excellent color prints are made from the color negative.

## EXAMPLE 6

Example 1 is repeated, but adding to the processing solution imbibant of Example 1 of 0.2 g./l. of 2-hydroxy-4-thiatetradecyl-trimethylammonium p-toluenesulfonate and 0.05 g./l. of 3-mercaptop-1,2,4-triazole. Excellent black-and-white positive, color negative and color print are obtained.

## 12

## EXAMPLE 7

Example 1 is repeated, but substituting 150 m./l. of 2,2'-iminodiethanol-SO<sub>2</sub> addition product (13% SO<sub>2</sub> by weight) for the 2-methylaminoethanol-SO<sub>2</sub> addition product in the web imbibant solution of Example 1. With this substitution, the pH of the imbibant solution is about 9.0. The quantity of solution imbibed under the conditions used in Example 1 is reduced from about 86 g./m.<sup>2</sup> to about 64 g./m.<sup>2</sup>. A useful image is produced in the web and a color negative, similar to that of Example 1, is produced.

## EXAMPLE 8

Example 3 is repeated, but substituting for the color developing agent used in Example 3, an equimolar amount of 4-amino-3-methyl-N-ethyl-N-β-sulfoethylaniline. Example 3 is again repeated, but substituting for the developing agent an equimolar amount of 4-amino-N-ethyl-N-β,γ-dihydroxypropylaniline. Example 3 is again repeated, but substituting for the developing agent used in Example 3 an equimolar amount of 4-amino-N-ethyl-N-(2-methoxyethyl)-m-toluidine-dihydrochloride. In each of the repeats, black-and-white positive image, color negatives and color prints are obtained of quality comparable to the quality obtained in Example 3.

## EXAMPLE 9

Example 1 is repeated, but using a conventional color negative film in which the emulsion layers are found to have a reticulation temperature of about 23° C. and a melting point of about 48° C. when measured as described herein previously. Upon separating the processing web from the processed color negative, the hydrophilic colloid layers of the color negative are found to be physically damaged by the web process and of no value. This example is outside our invention, since the hydrophilic colloid emulsion layers of the color negative material do not have reticulation temperatures above 65° C. and melting points above 85° C.

## EXAMPLE 10

Example 1 is repeated, but (1) using a conventional color negative film in which the emulsion layers are found to have a reticulation temperature of about 23° C. and a melting point of about 48° C. when measured as described herein previously before processing and (2) adding 2 g./l. of glutaraldehyde bisulfite addition complex to the imbibant solution used in Example 1. The gelatin layers in the color negative element and in the processing web are hardened during the fifteen-minute processing step in which the negative element and web are contacted so that when separated, the gelatin layers are found to have reticulation temperatures greater than 65° C. and melting points greater than 85° C. and there is no physical damage caused in the negative or web when they are separated. A good color negative is produced in the element which is used after the bleaching and fixing steps, to make a good color print as described in Example 1. Similarly, it can be shown that appropriate amounts of other hardening agents described herein previously are advantageously used in place of glutaraldehyde bisulfite in Example 10 to give good color negatives and silver positives.

## EXAMPLE 11

Example 1 is repeated, but using the direct-positive photographic silver halide emulsions with nondiffusible couplers described in Coatings 3, 2 and 1 in Example III in Illingsworth, U.S. Pat. 3,501,305, issued Mar. 17, 1970, in place of the red-sensitive layer, the green-sensitive layer and blue-sensitive layers, respectively, used in the element of immediate Example 1. The gelatin in the web and the gelatin in the layers of the direct-positive photographic element are hardened during manufacture so that they have reticulation temperatures greater than 65° C. and melting points greater than 85° C. The direct-positive

photographic element is exposed and processed as described in Example 1 to produce a silver negative image reproduction in the processing web and a silver positive and a dye positive image in the direct-positive photographic element. Removal of the silver and residual silver halide from the web-processed direct-positive color element leaves a good, stable color positive image.

## EXAMPLE 12

Example 11 is repeated, but (1) using direct-positive silver halide emulsion layers that have a reticulation temperature of about 23° C. and a melting point of about 48° C. when measured as described herein previously before processing and (2) adding 2 g./l. of glutaraldehyde bisulfite addition complex to the imbibant solution used in Example 1. The gelatin layers in the direct-positive element and in the processing web are hardened during the fifteen-minute processing step in which the direct-positive element and web are contacted so that when separated, the gelatin layers are found to have reticulation temperatures greater than 65° C. and melting points greater than 85° C. and there is no physical damage caused in the direct-positive or web when they are separated. A good color positive is produced in the element that is stabilized by removal of silver and residual silver halide as described in Example 1.

## EXAMPLE 13

Examples 1, 3, 10, 11 and 12 are repeated, except that the five-minute bleach step and the five-minute fix step are replaced by a combined ten-minute bleach-fix step, using a solution having the composition:

|                                                      |     |
|------------------------------------------------------|-----|
| G.                                                   |     |
| Ammonium ethylenedinitrilotetraacetato ferrate (III) | 145 |
| Ammonium thiosulfate                                 | 148 |
| Ammonium sulfite                                     | 12  |
| Water to 1 liter.                                    |     |

The color reproductions obtained in each instance are of the same excellent quality obtained in Examples 1, 3, 10, 11 and 12.

An alternative procedure for producing a black-and-white image in a web material and a dye image in a radiation-sensitive color material is as follows: The diffusion transfer process that has been described is used, but a developing agent or combination of developing agents that produce only silver images, rather than silver and dye images, in the color material are incorporated in the imbibant solution. The p-phenylenediamine type developing agent is omitted. Following the diffusion transfer step, the color material bearing a silver image is fixed to remove silver halide, and then treated with a rehalogenizing bleach to convert the silver image to silver halide. The silver halide image is given an overall white light exposure sufficient to completely fog the silver halide, and is then processed in a conventional color process, such as that described in Example 1 of U.S. Pat. 2,956,879 to produce dye images in the color material.

The invention has been described in detail with particular reference to certain preferred embodiments thereof, but it will be understood that variations and modifications can be effected within the spirit and scope of the invention.

We claim:

1. A color process for an imagewise-exposed photographic element for producing during a single processing step a silver and a dye image in said element and producing a transfer silver image in a hydrophilic colloid processing web coated on a separate support, said photographic element comprising a support coated on one side with at least one hydrophilic colloid layer containing dispersed silver halide grains and a non-diffusible dye-forming coupler that reacts with an oxidized aromatic primary amine color developing agent to produce a nondiffusible dye, said hydrophilic colloid in said processing web and in said element being hardened either during manufacture

or during process step (1) below to have a reticulation temperature greater than 65° C. and a melting point greater than 85° C., said process comprising the steps:

(1) contacting said hydrophilic colloid layer of the imagewise-exposed photographic element with said hydrophilic colloid processing web which contains silver precipitating agent, an alkali, an aromatic primary amine color developing agent and a silver halide solvent until substantially all developable silver halide grains in said photographic element are developed to a silver image and a nondiffusible dye image, and at least a part of the undeveloped silver halide grains in areas not color developed in said photographic element are dissolved by said silver halide solvent and transferred imagewise to said hydrophilic colloid processing web where a silver image is formed on said silver precipitating agent, said processing web containing a hardening agent when said hydrophilic colloid in said photographic element and said web are not hardened during manufacture;

(2) separating said processing web containing its silver image from said photographic element containing its silver and dye image and any residual undeveloped silver halide.

2. The process of claim 1 in which said hydrophilic colloid layer on said photographic element and on said processing web is gelatin.

3. A color process for an imagewise-exposed photographic element for producing during a single development step a silver and a dye image in said element and producing a transfer silver image in a hardened hydrophilic colloid processing web having a reticulation temperature greater than 65° C. and a melting point greater than 85° C. coated on a separate support, said photographic element comprising a support coated on one side with at least one hardened hydrophilic colloid layer having a reticulation temperature greater than 65° C. and a melting point greater than 85° C. containing dispersed silver halide grains and a nondiffusible dye-forming coupler that reacts with an oxidized aromatic primary amine color developing agent to produce a nondiffusible dye, said process comprising the steps:

(1) contacting said hydrophilic colloid layer of the photographic element with said hydrophilic colloid processing web which contains silver precipitating agent, an alkali, an aromatic primary amine color developing agent and a silver halide solvent until substantially all developable silver halide grains in said photographic element are developed to a silver image and a nondiffusible dye image, and at least a part of the undeveloped silver halide grains in areas not color developed in said photographic element are dissolved by said silver halide solvent and transferred imagewise to said hydrophilic colloid processing web where a silver image is formed on said silver precipitating agent, and

(2) separating said processing web containing its silver image from said photographic element containing its silver and dye image and any residual undeveloped silver halide.

4. A color process for an imagewise-exposed photographic element for producing during a single processing step a silver and a dye image in said element and producing a transfer silver image in a hydrophilic colloid processing web coated on a separate support, said photographic element comprising a support coated on one side with at least one hydrophilic colloid layer containing dispersed silver halide grains and a nondiffusible dye-forming coupler that reacts with an oxidized aromatic primary amine color developing agent to produce a nondiffusible dye, said process comprising the steps:

(1) contacting said hydrophilic colloid layer of the photographic element with said hydrophilic colloid

## 15

processing web which contains silver precipitating agent, an alkali, an aromatic primary amine color developing agent, a silver halide solvent and a hardening agent until substantially all developable silver halide grains in said photographic element are developed to a silver image and a nondiffusible dye image, and at least a part of the undeveloped silver halide grains in areas not color developed in said photographic element are dissolved by said silver halide solvent and transferred imagewise to said hydrophilic colloid processing web where a silver image is formed on said silver precipitating agent, and until said hardening agent has hardened said hydrophilic colloid in said photographic element and in said web so that it has a reticulation temperature greater than 65° C. and a melting point greater than 85° C.; and (2) separating said processing web containing its silver image from said photographic element containing its silver and dye image and any residual undeveloped silver halide.

5. A color process for an imagewise-exposed photographic element for producing a dye image in said element and producing a transfer silver image in a hardened hydrophilic colloid processing web having a reticulation temperature greater than 65° C. and a melting point greater than 85° C., said photographic element comprising a support coated on one side with at least one hardened hydrophilic colloid layer having a reticulation temperature greater than 65° C. and a melting point greater than 85° C. containing dispersed silver halide grains and a nondiffusible dye-forming coupler that reacts with an oxidized aromatic primary amine color developing agent to produce a nondiffusible dye, said process comprising the steps:

(1) contacting said hydrophilic colloid layer of the photographic element with said hydrophilic colloid processing web which contains silver precipitating agent, an alkali, an aromatic primary amine color developing agent and a silver halide solvent until substantially all developable silver halide grains in said photographic element are developed to a silver image and a nondiffusible dye image, and at least a part of the undeveloped silver halide grains in areas not color developed in said photographic element are dissolved by said silver halide solvent and transferred imagewise to said hydrophilic colloid processing web where a silver image is formed on said silver precipitating agent;

(2) separating said processing web containing its silver image from said photographic element containing its silver and dye image and any residual undeveloped silver halide;

(3) contacting the silver image and any residual silver halide in said photographic element from step (2) with a silver bleach bath comprising a photographic silver oxidizing agent until the silver is converted to a silver salt; and

(4) contacting said silver salt with a photographic fixing bath comprising a silver salt solvent until said silver salt is dissolved and diffuses from said photographic element so said dye image is unobstructed and made permanent.

6. A color process for an imagewise-exposed photographic element for producing a dye image in said element and producing a transfer silver image in a hardened hydrophilic colloid processing web, said photographic element comprising a support coated on one side with at least one hardened hydrophilic colloid layer having a reticulation temperature greater than 65° C. and a melting point greater than 85° C. containing dispersed silver halide grains and a nondiffusible dye-forming coupler that reacts with an oxidized aromatic primary amine color developing agent to produce a nondiffusible dye, said process comprising the steps:

(1) contacting said hydrophilic colloid layer of said

5

10

15

20

25

30

35

40

45

50

55

60

65

70

## 16

photographic element with said hydrophilic colloid processing web which contains silver precipitating agent, an alkali, an aromatic primary amine color developing agent and a silver halide solvent until substantially all developable silver halide grains in said photographic element are developed to a silver image and a nondiffusible dye image, and at least a part of the undeveloped silver halide grains in areas not color developed in said photographic element are dissolved by said silver halide solvent and transferred imagewise to said hydrophilic colloid processing web where a silver image is formed on said silver precipitating agent;

(2) separating said processing web containing its silver image from said photographic element containing its silver and dye image and any residual undeveloped silver halide; and

(3) contacting said silver image and any residual silver halide in said photographic element from step (2) with a combined bleach-and-fix solution comprising a silver oxidizing agent and a silver salt solvent until said silver and said silver salt are dissolved and diffused from said photographic element so said dye image is unobstructed and made permanent.

7. A color process for an imagewise-exposed photographic element for producing during a single processing step a silver negative and a color negative image in said element and producing a transfer silver positive image in a hydrophilic colloid processing web coated on a separate support, said photographic element comprising a support coated on one side with at least one hydrophilic colloid layer containing dispersed silver halide grains and a nondiffusible dye-forming coupler that reacts with an oxidized aromatic primary amine color developing agent to produce a non-diffusible dye, said hydrophilic colloid in said processing web and in said element being hardened either during manufacture or during process step (1) below to have a reticulation temperature greater than 65° C. and a melting point greater than 85° C., said process comprising the steps:

(1) contacting said hydrophilic colloid layer of the imagewise-exposed photographic element with said hydrophilic colloid processing web which contains silver precipitating agent, an alkali, an aromatic primary amine color developing agent and a silver halide solvent until substantially all developable silver halide grains in said photographic element are developed to a silver negative image and a nondiffusible dye negative image, and at least a part of the undeveloped silver halide grains in areas not color developed in said photographic element are dissolved by said silver halide solvent and transferred imagewise to said hydrophilic colloid processing web where a silver positive image is formed on said silver precipitating agent, said processing web containing a hardening agent when said hydrophilic colloid in said photographic element and said web are not hardened during manufacture; and

(2) separating said processing web containing its silver image from said photographic element containing its silver and dye image and any residual undeveloped silver halide.

8. A color process for an imagewise-exposed multi-layer, multicolor photographic element for producing during a single processing step a silver negative and a color negative image in said element and producing a transfer silver positive image in a hardened hydrophilic colloid processing web having a reticulation temperature greater than 65° C. and a melting point greater than 85° C. coated on a separate support, said photographic element comprising a support coated on one side with a first hardened hydrophilic colloid silver halide emulsion layer sensitive to light from a first region of the visible spectrum and a coupler that reacts with an oxidized aromatic primary amine color developing agent to form a

75

nondiffusible dye image of a first color, a second hardened hydrophilic colloid silver halide emulsion layer sensitive to a second region of the visible spectrum that is different from said first region and a second coupler that reacts with an oxidized aromatic primary amine color developing agent to form a nondiffusible dye image of a second color that is different from said first color dye, and a third hardened hydrophilic colloid silver halide emulsion layer sensitive to a third region of the visible spectrum that is different from said first region and said second region and a third coupler that reacts with oxidized aromatic primary amine color developing agent to form a nondiffusible dye image of a third color that is different from said first color and said second color, said emulsion layers each having a reticulation temperature greater than 65° C. and a melting point greater than 85° C., said process comprising the steps:

- (1) contacting said hydrophilic colloid layer of the photographic element with said hydrophilic colloid processing web which contains silver precipitating nuclei, an alkali, an aromatic primary amine color developing agent and a silver halide solvent until substantially all developable silver halide grains in said photographic element are developed to a silver negative image and a non-diffusible dye negative image, and at least a part of the undeveloped silver halide grains in areas not color developed in said photographic element are dissolved by said silver halide solvent and transferred imagewise to said hydrophilic colloid processing web where a silver positive image is formed on said silver precipitating nuclei; and
- (2) separating said processing web containing said silver positive image from said photographic element containing said silver negative and dye negative image and any residual undeveloped silver halide.

9. A color process for an imagewise-exposed multi-layer, multicolor photographic element for producing during a single processing step a silver negative and a dye negative image in said element and producing a corresponding transfer silver positive image in a hardened hydrophilic colloid processing web having a reticulation temperature greater than 65° C. and a melting point greater than 85° C. coated on a separate support, said photographic element comprising a support coated on one side with a hardened hydrophilic colloid layer containing red-sensitive silver halide grains and a nondiffusible coupler that reacts with an oxidized aromatic primary amine color developing agent to form a nondiffusible cyan dye image, a hardened hydrophilic colloid layer containing green-sensitive silver halide grains and a nondiffusible coupler that reacts with an oxidized aromatic primary amine color developing agent to form a nondiffusible magenta dye, a hardened hydrophilic colloid layer containing blue-sensitive silver halide grains and a nondiffusible coupler that reacts with an oxidized aromatic primary amine color developing agent to form a nondiffusible yellow dye, said hardened hydrophilic colloid layers in said photographic element each having a reticulation temperature greater than 65° C. and a melting point greater than 85° C., said process comprising the steps:

- (1) contacting said hydrophilic colloid layer of the photographic element with said hydrophilic colloid processing web which contains silver precipitating nuclei, an alkali, an aromatic primary amine color developing agent and a silver halide solvent until substantially all developable silver halide grains in said photographic element are developed to a silver negative image and a nondiffusible dye negative image, and at least a part of the undeveloped silver halide grains in areas not color developed in said photographic element are dissolved by said silver halide solvent and transferred imagewise to said hydrophilic colloid processing web where a silver positive

image is formed on said silver precipitating nuclei; and

(2) separating said processing web containing said silver positive image from said photographic element containing said silver negative and dye negative image and any residual undeveloped silver halide.

10. The process of claim 9 in which said hydrophilic colloid in said element and in said processing web is hardened gelatin.

11. A color process for an imagewise-exposed multi-layer, multicolor direct-positive photographic element for producing during a single processing step a silver positive and a color positive image in said element and producing a corresponding transfer silver negative image in a hardened hydrophilic colloid processing web having a reticulation temperature greater than 65° C. and a melting point greater than 85° C. coated on a separate support, said photographic element comprising a support coated on one side with a first hardened hydrophilic colloid direct-positive silver halide emulsion layer sensitive to light from a first region of the visible spectrum and a coupler that reacts with an oxidized aromatic primary amine color developing agent to form a nondiffusible dye image of a first color, a second hardened hydrophilic colloid direct-positive silver halide emulsion layer sensitive to a second region of the visible spectrum that is different from said first region and a second coupler that reacts with an oxidized aromatic primary amine color developing agent to form a nondiffusible dye image of a second color that is different from said first color dye, and a third hardened hydrophilic colloid direct-positive silver halide emulsion layer sensitive to a third region of the visible spectrum that is different from said first region and said second region and a third coupler that reacts with oxidized aromatic primary amine color developing agent to form a nondiffusible dye image of a third color that is different from said first color and said second color, said emulsion layers each having a reticulation temperature greater than 65° C. and a melting point greater than 85° C., said process comprising the steps:

- (1) contacting said hydrophilic colloid layer of the photographic element with said hydrophilic colloid processing web which contains silver precipitating nuclei, an alkali, an aromatic primary amine color developing agent and a silver halide solvent until substantially all developable silver halide grains in said photographic element are developed to a silver positive image and a non-diffusible dye positive image, and at least a part of the undeveloped silver halide grains in areas not color developed in said photographic element are dissolved by said silver halide solvent and transferred imagewise to said hydrophilic colloid processing web where a silver negative image is formed on said silver precipitating nuclei; and
- (2) separating said processing web containing said silver negative image from said photographic element containing said silver positive and dye positive image and any residual undeveloped silver halide.

12. A color process for an imagewise-exposed multi-layer, multicolor direct-positive photographic element for producing during a single processing step a silver positive and a dye positive image in said element and producing a corresponding transfer silver negative image in a hardened hydrophilic colloid processing web having a reticulation temperature greater than 65° C. and a melting point greater than 85° C. coated on a separate support, said photographic element comprising a support coated on one side with a hardened hydrophilic colloid layer containing red-sensitive direct-positive silver halide grains and a nondiffusible coupler that reacts with an oxidized aromatic primary amine color developing agent to form a nondiffusible cyan dye image, a hardened hydrophilic colloid layer containing green-sensitive direct-positive silver halide grains and a nondiffusible coupler that reacts with an oxidized aromatic primary amine

color developing agent to form a nondiffusible magenta dye, a hardened hydrophilic colloid layer containing blue-sensitive direct-positive silver halide grains and a nondiffusible coupler that reacts with an oxidized aromatic primary amine color developing agent to form a nondiffusible yellow dye, said hardened hydrophilic colloid layers in said photographic element each having a reticulation temperature greater than 65° C. and a melting point greater than 85° C., said process comprising the steps:

- (1) contacting said hydrophilic colloid layer of the photographic element with said hydrophilic colloid processing web which contains silver precipitating nuclei, an alkali, an aromatic primary amine color developing agent and a silver halide solvent until substantially all developable silver halide grains in said photographic element are developed to a silver positive image and a nondiffusible dye positive image, and at least a part of the undeveloped silver halide grains in areas not color developed in said photographic element are dissolved by said silver halide solvent and transferred imagewise to said hydrophilic colloid processing web where a silver negative image is formed on said silver precipitating nuclei; and
- (2) separating said processing web containing said silver negative image from said photographic element containing said silver positive and dye positive image and any residual undeveloped silver halide.

13. The process of claim 12 in which said hydrophilic colloid in said element and in said processing web is hardened gelatin.

14. The process of claim 6 in which said hydrophilic colloid processing web contains a p-phenylenediamine color developing agent and an amine-sulfur dioxide addition product as the alkali and silver halide solvent.

15. The process of claim 6 in which said hydrophilic colloid processing web contains a solution containing in the range of from about 2 g./l. to about 100 g./l. of a color developing agent selected from the class consisting of

4-amino-3-methyl-N-ethyl-N-β-hydroxyethylaniline sulfate,  
4-amino-3-methoxy-N-β-hydroxyethylaniline hydrochloride,  
4-amino-N-ethyl-N-β-hydroxyethylaniline hydrochloride,  
4-amino-3-methyl-N-ethyl-N-β-sulfoethylaniline,  
4-amino-N-ethyl-N-β-γ-dihydroxypropylaniline and  
4-amino-N-ethyl-N-(2-methoxyethyl)-m-toluidine dihydrochloride

and contains in the range of from about 5 g./l. to about 300 g./l. of 2-methylaminoethanol-sulfur dioxide addition product and said solution has a pH in the range of from about 8.5 to about 11.5.

16. A color process for an imagewise-exposed multi-layer, multicolor photographic element for producing during a single processing step a silver and a dye image in said element and producing a transfer silver image in a hardened gelatin processing web coated on a separate support, said photographic element comprising a support coated on one side with a hardened gelatin layer containing red-sensitive silver bromoiodide grains and a nondiffusible coupler that reacts with an oxidized aromatic primary amine color developing agent to form a nondiffusible cyan dye image, a hardened gelatin layer containing green-sensitive silver bromoiodide grains and a nondiffusible coupler that reacts with an oxidized aromatic primary amine color developing agent to form a nondiffusible magenta dye, a hardened gelatin layer containing blue-sensitive silver bromoiodide grains and a nondiffusible coupler that reacts with an oxidized aromatic primary amine color developing agent to form a nondiffusible yellow dye, each of said hardened gelatin layers in said photographic element having a reticulation

temperature of 83° C. and a melting point greater than 100° C., said process comprising the steps:

- (1) contacting said gelatin layer of said photographic element with said gelatin layer of said processing web which contains a nickel sulfide-silver iodide silver precipitating nuclei; an aqueous alkaline solution containing 2-methylaminoethanol —SO<sub>2</sub> addition product, 4-amino-3-methyl-N-ethyl-N-β-hydroxyethylaniline sulfate and sodium thiosulfate to convert substantially all developable silver bromoiodide grains to a silver image and a dye image in said photographic element, to dissolve in said 2-methylaminoethanol —SO<sub>2</sub> addition product and said sodium thiosulfate at least a part of the undeveloped silver bromoiodide grains in areas not color developed in said photographic element and to transfer said dissolved silver bromoiodide imagewise to said silver precipitating nuclei and form a corresponding silver image on said nuclei; and
- (2) separating said processing web containing its silver image from said photographic element containing its corresponding silver image, dye image and any residual undeveloped silver bromoiodide grains.

17. A color process for an imagewise-exposed multi-layer, multicolor photographic element for producing during a single processing step a silver and a dye image in said element and producing a transfer silver image in a hardened gelatin processing web having a reticulation temperature greater than 65° C. and a melting point greater than 85° C., coated on a separate support, said photographic element comprising a support coated on one side with a hardened gelatin layer containing red-sensitive silver bromoiodide grains and a non-diffusible coupler that reacts with an oxidized aromatic primary amine color developing agent to form a nondiffusible magenta dye, a hardened gelatin layer containing green-sensitive silver bromoiodide grains and a nondiffusible coupler that reacts with an oxidized aromatic primary amine color developing agent to form a nondiffusible cyan dye image, a hardened gelatin layer containing blue-sensitive silver bromoiodide grains and a nondiffusible coupler that reacts with an oxidized aromatic primary amine color developing agent to form a nondiffusible yellow dye, each of said hardened gelatin layers in said photographic element having a reticulation temperature of 83° C. and a melting point of greater than 100° C., said process comprising the steps:

- (1) contacting said gelatin layer of said photographic element with said gelatin layer of said processing web which contains nickel sulfide-silver iodide silver precipitating nuclei, an aqueous alkaline solution containing 2 - methylaminoethanol —SO<sub>2</sub> addition product and 4-amino - 3 - methoxy-N-ethyl-N-β-hydroxyethylaniline hydrochloride to convert substantially all developable silver bromoiodide grains to a silver image and a dye image in said photographic element, to dissolve in said 2-methylaminoethanol —SO<sub>2</sub> addition product at least a part of the undeveloped silver bromoiodide grains in areas not color developed in said photographic element and to transfer said dissolved silver bromoiodide imagewise to said silver precipitating nuclei and form a corresponding silver image in said nuclei; and
- (2) separating said processing web containing its silver image from said photographic element containing its corresponding silver image, said dye image and any residual undeveloped silver bromoiodide grains.

18. A color process for an imagewise-exposed multi-layer, multicolor photographic element for producing during a single processing step a silver negative and a dye negative image in said element and producing a transfer silver positive image in a hardened gelatin processing web coated on a separate support, said photographic element comprising a support coated on one side with a hardened gelatin layer containing red-sensitive silver bromoiodide grains and a nondiffusible coupler that reacts with an

21

oxidized aromatic primary amine color developing agent to form a nondiffusible cyan dye image, a hardened gelatin layer containing green-sensitive silver bromoiodide grains and a nondiffusible coupler that reacts with an oxidized aromatic primary amine color developing agent to form a nondiffusible magenta dye, a hardened gelatin layer containing blue-sensitive silver bromoiodide grains and a nondiffusible coupler that reacts with an oxidized aromatic primary amine color developing agent to form a nondiffusible yellow dye, each of said hardened gelatin layers in said photographic element having a reticulation temperature of 83° C. and a melting point greater than 100° C., said process comprising the steps:

- (1) contacting said gelatin layer of said photographic element for fifteen minutes at 20° C. with said gelatin layer of said processing web which contains 20.4 g./m.<sup>2</sup> of nickel sulfide-silver iodide silver precipitating nuclei; an aqueous solution of pH 10.0 containing 100 ml./l. of 2-methylaminoethanol —SO<sub>2</sub> addition product with 30% SO<sub>2</sub>, 40 g./l. of 4-amino-3-methyl-N-ethyl-N-β-hydroxyethylaniline sulfate and 10 g./l. of sodium thiosulfate to convert substantially all developable silver bromoiodide grains to a silver negative image and a dye negative image in said photographic element, to dissolve in said 2-methylaminoethanol —SO<sub>2</sub> addition product and said sodium thiosulfate at least a part of the undeveloped silver bromoiodide grains in areas not color developed in said photographic element and to transfer said dissolved silver bromoiodide imagewise to said silver precipitating nuclei and form a corresponding silver positive image on said nuclei; and
- (2) separating said processing web containing said silver positive image from said photographic element containing said silver negative image, said dye negative image and any residual undeveloped silver bromoiodide grains.

19. A color process for an imagewise-exposed multilayer, multicolor photographic element for producing during a single processing step a silver negative and a dye negative image in said element and producing a transfer silver positive image in a hardened gelatin processing web having a reticulation temperature greater than 65° C. and melting point greater than 85° C., coated on a separate support, said photographic element comprising a support coated on one side with a hardened gelatin layer containing red-sensitive silver bromoiodide grains and a nondiffusible coupler that reacts with an oxidized aromatic primary amine color developing agent to form

22

a nondiffusible cyan dye image, a hardened gelatin layer containing green-sensitive silver bromoiodide grains and a nondiffusible coupler that reacts with an oxidized aromatic primary amine color developing agent to form a nondiffusible magenta dye, a hardened gelatin layer containing blue-sensitive silver bromoiodide grains and a nondiffusible coupler that reacts with an oxidized aromatic primary amine color developing agent to form a nondiffusible yellow dye, each of said hardened gelatin layers in said photographic element having a reticulation temperature of 83° C. and a melting point of greater than 100° C., said process comprising the steps:

- (1) contacting said gelatin layer of said photographic element for ten minutes at 20° C. with said gelatin layer of said processing web which contains 20.4 g./m.<sup>2</sup> of nickel sulfide-silver iodide silver precipitating nuclei, an aqueous solution of pH 10.1 containing 90 ml./l. of 2-methylaminoethanol —SO<sub>2</sub> addition product with 7% SO<sub>2</sub> and 15 g./l. of 4-amino-3-methoxy-N-ethyl-N-β-hydroxyethylaniline hydrochloride to convert substantially all developable silver bromoiodide grains to a silver negative image and a dye negative image in said photographic element, to dissolve in said 2-methylaminoethanol —SO<sub>2</sub> addition product at least a part of the undeveloped silver bromoiodide grains in areas not color developed in said photographic element and to transfer said dissolved silver bromoiodide imagewise to said silver precipitating nuclei and form a corresponding silver positive image on said nuclei; and
- (2) separating said processing web containing said silver positive image from said photographic element containing said silver negative image, said dye negative image and any residual undeveloped silver bromoiodide grains.

#### References Cited

#### UNITED STATES PATENTS

|           |        |                  |       |         |
|-----------|--------|------------------|-------|---------|
| 2,712,995 | 7/1955 | Weyde            | ----- | 96—3    |
| 3,243,294 | 3/1966 | Barr             | ----- | 96—3    |
| 3,179,517 | 4/1965 | Tregillus et al. | ----- | 96—29 R |

NORMAN G. TORCHIN, Primary Examiner

A. T. SURO PICO, Assistant Examiner

U.S. Cl. X.R.

96—29 D, 29 R, 60 R, 60 BF, 64